# EUROPEAN PATENT SPECIFICATION

(11) **EP 0 460 008 B1**
(45) Date of publication and mention of the grant of the patent: **05.06.1996**
(21) Application number: 90903197.3
(22) Date of filing: 14.02.1990
(51) Int. Cl.: G03C 7/384, G03C 7/26

(54) **THE USE OF PYRAZOLO-TRIAZOLE PHOTOGRAPHIC COLOUR COUPLERS**
VERWENDUNG PYRAZOLTRIAZOL-FOTOGRAFISCHER FARBKUPPLER
EMPLOI DE COUPLEURS DE COULEUR PHOTOGRAPHIQUES DE PYRAZOLO-TRIAZOLE

(30) Priority: 22.02.1989 GB 8904004
(43) Date of publication of application: 11.12.1991
(73) Proprietor: KODAK LIMITED, Hemel Hempstead Herts, HP1 1JU (GB); EASTMAN KODAK COMPANY, Rochester, New York 14650-2201 (US)
(72) Inventor: THOMAS, Brian, Bucks HP9 1LF (GB); LEYSHON, Llewellyn, James, Watford, Herts WD1 3HW (GB); CLARKE, David, Herts WD2 4HL (GB)
(74) Representative: Baron, Paul Alexander Clifford
(86) International application number: GB9000232
(87) International publication number: WO9010253

(56) References cited:
- EP-A- 0 273 712
- EP-A- 0 325 276
- EP-A- 0 326 406
- US-A- 4 766 057
- Derwent's abstract, No 87-339618/48, JP 62246054, publ. week 8748, Dialog Information Service, file 351, WPI

## Description

This invention relates to the use of 1H-pyrazolo[1,5-b]-1,2,4-triazole couplers in photographic materials.

1H-Pyrazolo[1,5,-b]-1,2,4-triazole couplers have been described in, for example, US Patent 4,621,046. In European Patent Specification 0,177,765 such a coupler having the formula: is incorporated in a silver chlorobromide (50% bromide) emulsion. The coupler is said to provide dye images of good fastness and freedom from yellow stain.

Similarly couplers containing a tertiary butyl group in the 2- or 6-position are disclosed in European Patent Specifications 0 326 406 and 0 271 712, the former document belonging to the state of the art by virtue of Article 54(3) EPC.

Currently photographic colour paper processable in the RA4 process is comprised of silver halide emulsions having at least 80% silver chloride and preferably substantially pure silver chloride. Most 1H-pyrazolo[1,5-b]-1,2,4-triazole couplers when incorporated into silver chloride emulsions provide photographic materials having poor raw stock keeping properties. That is, the material when stored after manufacture but before exposure and processing, shows significantly increased Dₘᵢₙ compared to freshly coated materials.

Accordingly the present invention is directed to the use of 1H-pyrazolo[1,5-b]-1,2,4- triazole couplers containing a tertiary carbon group in the 2- or 6- position of the coupler nucleus in photographic silver halide materials of which the halide comprises more than 80% chloride, in order to improve raw stock stability.

Preferably the silver halide emulsion comprises at least 90% silver chloride especially substantially pure silver chloride.

The preferred couplers have the formula
wherein R¹ and R³ are each an alkyl or substituted alkyl group, and
R² is a hydrogen or a coupling off group, at least one of R¹ and R³ comprising a group of the formula:
wherein R⁴, R⁵ and R⁶ are individually a halogen atom or an alkyl, cycloakyl, amino, aryl, cyano, nitro, heterocyclic or -L-R⁷ group
wherein L is a linking group and R⁷ is an alkyl, aryl, heterocyclic group and
wherein any two of R⁴, R⁵ and R⁶ can form a heterocyclic or alicyclic ring,
any of the groups R⁴, R⁵ and R⁶ being optionally substituted, all of the above groups and substituents being such that they do not adversely affect the desired properties of the coupler.

In the above general formula when R¹ or R³ are a tertiary alkyl group they preferably contain 4-8 carbon atoms and may be t-butyl, t-pentyl or t-octyl. R¹ and R³ may otherwise contain 1-25 carbon atoms and may comprise a ballast group to render the coupler non-diffusible in photographic layers.

Examples of R⁴, R⁵ and R⁶ are chlorine, bromine and fluorine; alkyl groups containing 1 to 20 carbon atoms, for example, methyl, ethyl, propyl, butyl, pentyl, ethylhexyl and eicosyl; cyclohexyl and cyclopentyl; dioctylamino, dimethylamino and dodecylamino; aryl containing 6 to 20 carbon atoms,for example, phenyl, naphthyl and mesityl; cyano; nitro; a heterocyclic group comprised of atoms selected from carbon, oxygen, nitrogen and sulphur atoms necessary to complete a 5- or 6-membered ring, for example, pyrrolyl, oxazolyl and pyridyl.

Examples of L are: O, S, CO, CO₂, SO₂, SO, in which R⁸ and R⁹ are individually hydrogen, alkyl, such as alkyl containing 1 to 30 carbon atoms, for example, methyl, ethyl, propyl, butyl or eicosyl, or aryl, such as aryl containing 6 to 20 carbon atoms, for example, phenyl or naphthyl; or a heterocyclic group comprised of atoms selected from carbon, nitrogen, oxygen, and sulphur atoms necessary to complete a 5- or 6-member heterocyclic ring, for example, pyrrolyl, oxazolyl and pyridyl.

Examples of R⁷ are an alkyl containing 1 to 30 carbon atoms, for example, methyl, ethyl, propyl, butyl, pentyl and eicosyl; aryl, such as aryl containing 6 to 20 carbon atoms, for example, phenyl and napthyl; or a heterocyclic group, such as a 5- or 6-membered heterocyclic group comprised of atoms selected from carbon, nitrogen, oxygen and sulphur atoms, for example an oxazole, pyridine, pyrrole or thiophene ring.

When any two of R⁴, R⁵ and R⁶ form a heterocyclic ring this may be an oxazole, pyridine, pyrrole and thiophene; or when they form an alicyclic ring system, this may be cyclohexyl, norbornyl or adamantyl.

The coupling-off group R² may be a halogen atom or an aryloxy or arylthio group.

The couplers used in the present invention may be prepared by methods known in the art.

Typically, the couplers are associated with a silver halide emulsion layer coated on a support to form a photographic element. As used herein, the term "associated with" signifies that the coupler is incorporated in the silver halide emulsion layer or in a layer adjacent thereto where, during processing, it is capable of reacting with silver halide development products.

The photographic elements can be single colour elements or multicolour elements. In a multicolour element, the magenta dye-forming couplers used in this invention would usually be associated with a green-sensitive emulsion, although they could be associated with an emulsion sensitised to a different region of the spectrum, or with a panchromatically sensitised, orthochromatically sensitised or unsensitised emulsion. Multicolour elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art.

A typical multicolour photographic element comprises a support bearing yellow, magenta and cyan dye image-forming units comprising at least one blue-, green- or red-sensitive silver halide emulsion layer having associated therewith at least one yellow, magenta or cyan dye-forming coupler respectively, at least one of the magenta dye-forming couplers being a coupler of this invention. The element can contain additional layers, such as filter and barrier layers.

In the following discussion of suitable materials for use in the emulsions and elements of this invention, reference will be made to Research Disclosure, December 1978, Item 17643, published by Industrial Opportunities Ltd., The Old Harbourmaster's, 8 North Street, Emsworth, Hants P010 7DD, U.K. This publication will be identified hereafter as "Research Disclosure".

The silver halide emulsion employed in the elements of this invention can be either negative-working or positive-working. Suitable emulsions and their preparation are described in Research Disclosure Sections I and II and the publications cited therein. Suitable vehicles for the emulsion layers and other layers of elements of this invention are described in Research Disclosure Section IX and the publications cited therein.

In addition to the couplers of this invention, the elements of the invention can include additional couplers as described in Research Disclosure Section VII, paragraphs D, E, F and G and the publications cited therein. The couplers of this invention and any additional couplers can be incorporated in the elements and emulsions as described in Research Disclosures of Section VII, paragraph C and the publications cited therein.

The photographic elements of this invention or individual layers thereof, can contain brighteners (see Research Disclosure Section V), antifoggants and stabilisers (see Research Disclosure Section VI), antistain agents and image dye stabiliser (see Research Disclosure Section VII, paragraphs I and J), light absorbing and scattering materials (see Research Disclosure Section VIII), hardeners (see Research Disclosure Section XI), plasticisers and lubricants (see Research Disclosure Section XII), antistatic agents (see Research Disclosure Section XIII), matting agents (see Research Disclosure Section XVI) and development modifiers (see Research Disclosure Section XXI).

The photographic elements can be coated on a variety of supports as described in Research Disclosure Section XVII and the references described therein.

Photographic elements can be exposed to actinic radiation, typically in the visible region of the spectrum, to form a latent image as described in Research Disclosure Section XVIII and then processed to form a visible dye image as described in Research Disclosure Section XIX. Processing to form a visible dye image includes the step of contacting the element with a colour developing agent to reduce developable silver halide and oxidise the colour developing agent. Oxidised colour developing agent in turn reacts with the coupler to yield a dye.

Preferred colour developing agents are p-phenylene diamines. Especially preferred are 4-amino-3-methyl-N,N-diethylaniline hydrochloride, 4-amino-3-methyl-N-ethyl-N-β-(methanesulphonamido)-ethylaniline sulphate hydrate, 4-amino-3-methyl-N-ethyl-N-β-hydroxyethylaniline sulphate, 4-amino-3-β-(methanesulphonamido)ethyl-N,N-diethylaniline hydrochloride and 4-amino-N-ethyl-N-(2-methoxyethyl)-m-toluidine di-p-toluene sulphonate.

With negative-working silver halide emulsions this processing step leads to a negative image. To obtain a positive (or reversal) image, this step can be preceded by development with a non-chromogenic developing agent to develop exposed silver halide, but not form dye, and then uniform fogging of the element to render unexposed silver halide developable. Alternatively, a direct positive emulsion can be employed to obtain a positive image.

Development is followed by the conventional steps of bleaching, fixing, or bleach-fixing, to remove silver and silver halide, washing and drying.

The following examples are included for a better understanding of the invention.

### EXAMPLE 1

Couplers were dispersed and coated as follows. The test coupler (3.0 mmol), dissolved in half its weight of di-n-butyl phthalate and ethyl acetate (2.0g), was dispersed in aqueous gelatin (36g, 12.5%) using ultrasonic agitation. The gelatin solution contained a small amount (0.5%) of di-isopropyl-naphthalene sulphonic acid (sodium salt) as a surfactant. The resultant coupler dispersion was diluted to 200g with water and mixed with a green-sensitised silver chloride photographic emulsion (100g, 1.49% Ag, 4.5% gel).
The mixture was spread on a resin-coated paper support to give a layer of the following composition:

| | |
|---|---|
| Ag | 0.267g.m⁻² |
| Coupler | 0.54mmol.m⁻² |
| Gelatin | 1.61g.m⁻² |

A protective gel supercoat containing hardener was applied to the coating.

Sample strips of the coatings were exposed through a step tablet (density range 0-3, 0.15 increments) and developed in standard "KODAK" RA-4 process solutions.

Sample strips from each coating were exposed and processed with RA4 chemistry within a few days of coating. Similar strips were put aside in a light-tight box and stored under ambient conditions for 29 weeks before exposure and processing.

The sensitometric parameters of the two sets of coatings were measured. It was observed that the stored coatings showed significantly higher Dmin values than the freshly processed coatings. However, the increase in Dmin was much smaller for the 6-t-Bu substituted examples Ib and Id than for their analogous 6-Me couplers,Ia and Ic. (See Table below)

### EXAMPLE 2

Couplers IIa and IIb were examined as described in Example 1, except that the storage time was reduced to 17 weeks. The sensitometric data shown below confirmed the advantage of the 6-t-Bu substituent.

| Coupler | R | Fresh D.min | Stored D.min |
|---|---|---|---|
| IIa | Me | 0.11 | 0.20 |
| IIb | t-Bu | 0.10 | 0.12 |

Couplers IIIa and IIIb were dispersed with the stabilising compound IV in the following proportions:

| | |
|---|---|
| Coupler | 2 |
| Stabiliser | 1 |
| Solvent (dibutyl phthalate) | 3 |

The dispersions were coated with a green sensitive silver chloride emulsion so as to give the following coverages:

| | |
|---|---|
| Coupler: | 0.57mmole.m⁻² |
| Silver: | 2.4mmole.m⁻² |

One pair of sample strips from each coating was incubated for 7 days at 50°C, 50%RH in the dark for comparison with an identical pair stored at ambient temperature. Both pairs were step wedge exposed and processed (RX4). The sensitometric data shown below show that the strips stored at elevated temperature showed a much greater Dmin than those stored at room temperature, but the difference was dramatically lower for the 6-t-Bu example (IIIb) than for IIIa.

| Coupler | R | ΔDmin (inc - fresh) |
|---|---|---|
| IIIa | Me | +1.39 |
| IIIb | t-Bu | +0.28 |

## Claims

1. The use of 1H-pyrazolo[1,5-b]-1,2,4-triazole couplers containing a tertiary carbon group in the 2- or 6- position of the coupler nucleus in photographic silver halide materials of which the halide comprises more than 80% chloride, in order to improve raw stock stability.

2. The invention as claimed in Claim 1 in which the coupler has the formula:
wherein R¹ and R³ are each an alkyl or substituted alkyl group, and
R² is a hydrogen or a coupling off group, at least one of R¹ and R³ comprising a tertiary carbon group of the formula:
wherein R⁴, R⁵ and R⁶ are individually a halogen atom or an alkyl, cycloakyl, amino, aryl, cyano, nitro, heterocyclic or -L-R⁷ group
wherein L is a linking group and R⁷ is an alkyl, aryl, heterocyclic group and
wherein any two of R⁴, R⁵ and R⁶ can form a heterocyclic or alicyclic ring,
any of the groups R⁴, R⁵ and R⁶ being optionally substituted, all of the above groups and substituents being such that they do not adversely affect the desired properties of the coupler.

3. The invention as claimed in Claim 2 in which R¹ or R³ is a tertiary alkyl group containing 4-8 carbon atoms.

4. The invention as claimed in any of Claims 1-3 in which the coupler comprises a coupling-off group which is a halogen atom or an aryloxy or arylthio group.

5. The invention as claimed in any of Claims 1-4 in which the emulsion is substantially pure silver chloride.

## Patentansprüche

1. Verwendung von 1H-Pyrazolo[1,5-b]-1,2,4-triazol-Kupplern mit einer tertiären Kohlenstoffgruppe in der 3- oder 6-Position des Kupplerkernes in photographischen Silberhalogenidmaterialien, in denen das Halogenid zu mehr als 80 % aus Chlorid besteht, um die Stabilität des Rohmaterials zu verbessern.

2. Die Erfindung gemäß Anspruch 1, worin der Kuppler die Formel hat:
worin R¹ und R³ jeweils eine Alkyl- oder substituierte Alkylgruppe darstellen, und
R² steht für ein Wasserstoffatom oder eine abkuppelnde Gruppe, wobei mindestens eine der Gruppen R¹ und R³ eine tertiäre Kohlenstoffgruppe der Formel ist:
worin R⁴, R⁵ und R⁶ einzeln stehen für ein Halogenatom oder eine Alkyl-, Cycloalkyl-, Amino-, Aryl-, Cyano-, Nitro- oder heterocyclische Gruppe oder eine Gruppe -L-R⁷,
worin L für eine verbindende Gruppe steht, und
R⁷ steht für eine Alkyl-, Aryl- oder heterocyclische Gruppe, und worin beliebige zwei von R⁴, R⁵ und R⁶ einen heterocyclischen oder alicyclischen Ring bilden können,
wobei jede der Gruppen R⁴, R⁵ und R⁶ gegebenenfalls substituiert sein kann, und wobei sämtliche der obigen Gruppen und Substituenten derart beschaffen sind, daß sie die erwünschten Eigenschaften des Kupplers nicht nachteilig beeinflussen.

3. Die Erfindung nach Anspruch 2, worin R¹ oder R³ für eine tertiäre Alkylgruppe mit 4 - 8 Kohlenstoffatomen stehen.

4. Die Erfindung nach einem der Ansprüche 1 - 3, worin der Kuppler eine abkuppelnde Gruppe aufweist, die aus einem Halogenatom oder einer Aryloxy- oder Arylthiogruppe besteht.

5. Die Erfindung nach einem der Ansprüche 1 - 4, worin die Emulsion eine praktisch reine Silberchloridemulsion ist.

## Revendications

1. Utilisation de coupleurs 1H-pyrazolo[1,5-b]-1,2,4-triazole contenant un groupe carbone tertiaire en position 2 ou 6 du noyau de coupleur dans des produits photographiques aux halogénures d'argent dans lesquels l'halogénure est constitué de plus de 80 % de chlorure, afin d'améliorer la stabilité du papier vierge.

2. Invention telle que revendiquée dans la revendication 1, dans laquelle le coupleur est représenté par la formule : où :
R¹ et R³ sont chacun un groupe alkyle ou alkyle substitué, et
R² est un hydrogène ou un groupe se séparant au couplage, au moins l'un des groupes R¹ et R³ comprenant un groupe carbone tertiaire de formule :
où :
R⁴, R⁵ et R⁶ sont individuellement un atome d'halogène, ou un groupe alkyle, cycloalkyle, amino, aryle, cyano, nitro, hétérocyclique ou -L-R'
où L est un groupe de liaison et
R' est un groupe alkyle, aryle, hétérocyclique et où l'un quelconque des deux groupes R⁴, R⁵ et le groupe R⁶ peuvent former un hétérocycle ou un cycle alicyclique,
l'un quelconque des groupes R⁴, R⁵ et R⁶ étant éventuellement substitué, tous les autres groupes et substituants précédents étant conçus de telle manière qu'ils n'influencent pas défavorablement les propriétés désirées du coupleur.

3. Invention telle que revendiquée dans la revendication 2, dans laquelle R¹ ou R³ est un groupe alkyle tertiaire de 4 à 8 atomes de carbone.

4. Invention telle que revendiquée dans l'une quelconque des revendications 1 à 3, dans laquelle le coupleur comprend un groupe se séparant au couplage qui est un atome d'halogène ou un groupe aryloxy ou arylthio.

5. Invention telle que revendiquée dans l'une quelconque des revendications 1 à 4, dans laquelle l'émulsion est constituée de chlorure d'argent pratiquement pur.
